

## UNITED STATES PATENT OFFICE

2,616,797

ALLOY FOR THE PREPARATION OF  
TITANIUM-BORON STEEL

Viatcheslav V. Efimoff, Niagara Falls, N. Y., assignor to National Lead Company, New York, N. Y., a corporation of New Jersey

No Drawing. Continuation of application Serial No. 95,573, May 26, 1949. This application December 19, 1950, Serial No. 201,700

3 Claims. (Cl. 75—124)

1

This invention relates to alloys containing titanium, boron, and aluminum which are particularly adapted for use in the manufacture of titanium-boron steels.

It has been previously known that steels containing about 0.3 to 0.5% titanium and 0.01 to 0.03% boron are characterized by superior resistance to load at moderately high temperatures. Such steels may be manufactured by adding to molten steel, after de-oxidizing, suitable amounts of metallic titanium and metallic boron, which preferably, are added in the form of ferro-alloys. At the temperatures at which these alloys are added to the steel, loss by oxidation of the added elements, particularly the titanium, is, to some degree, inevitable. It is helpful, therefore, to also add a de-oxidizing agent such as aluminum which improves the recovery of the added titanium and boron by protecting them from loss by oxidation, aluminum being more readily oxidized than either of these metals. The presence of aluminum has also been found to decrease the fusion point and improve the solubility (in molten steel) of ferro-titanium alloys. However, even under such conditions, the recoveries of titanium and boron have been difficult to predict with sufficient accuracy to insure the proper proportions of these added alloy elements in the final finished steel.

It is, therefore, the object of the present invention to provide a single alloy to be added to steel which will provide titanium and boron in proper proportions and which will insure high, uniform, predictable recoveries of these metals in finished steel. It is another object of this invention to provide a more efficient and economical method for production of titanium-boron alloy steel. These and other objects of the invention will be apparent from the following description thereof.

This invention in its broadest aspects contemplates provision of an alloy consisting of from about 35% to 45% of titanium, from about 1.5% to 2.8% boron, from about 8% to 15% aluminum and the remainder substantially all iron and incidental impurities. The impurities may include not more than an insignificant percentage of carbon, about 0.1%, for reasons hereinafter explained in more detail. Such an alloy when added to molten steel, after de-oxidation, will produce titanium-boron steel in which the titanium recovery will be about 80% and the boron recovery about 90%.

For illustration of a suitable method for preparation of an alloy according to this invention, the following example is shown:

2

## Example 1

A mixture of the following:

- 46.5 lbs. calcined granular ilmenite
- 5 22 lbs. refined granular rutile
- 36 lbs. pure grained aluminum
- 6 lbs. fused boric acid
- 10 lbs. sodium chlorate
- 1 lb. fluospar
- 10 with the following starting mix on top:
- 2 lbs. calcined granular ilmenite
- 1 lb. pure grained aluminum
- 0.5 lb. sodium chlorate
- 15 was ignited to produce a titanium-boron-aluminum ferro alloy by thermit reaction.

As a result of this reaction, 30 pounds of alloy

containing 38.04% titanium, 14.39% aluminum,

2.61% boron, 1.08% silicon, 0.07% carbon and the

remainder substantially all iron, was obtained

and separated from the slag.

An alternative method for preparation of the alloy of this invention employs ferrosilicon, preferably high grade ferrosilicon e. g. 94% Si, in the ignited mixture which improves the efficiency of the thermit reaction and therefore promotes better recovery of the alloy ingredients. Under these conditions, alloys containing aluminum in the lower ranges, that is 7 to 10%, may be produced. The amount of ferrosilicon in the original mixture should be such that not more than 4% silicon will be present in the product alloy, and in such amounts this element will not significantly affect the action or the usefulness of the alloy since the amount of silicon introduced into treated steel will have a negligible effect on the properties thereof.

An illustration of the manufacture of the alloy of this invention employing ferrosilicon in the starting mix is shown below.

## Example 2

A mixture of the following:

- 66 lbs. calcined granular ilmenite (61½% TiO<sub>2</sub>)
- 45 8 lbs. refined granular rutile
- 34 lbs. pure grained aluminum
- 6 lbs. fused boric acid
- 5 lbs. sodium chlorate
- 1 lb. fluospar
- 50 ½ lb. ferro silicon (94% Si)
- with the following starting mix on top:
- 1½ lbs. calcined granular ilmenite (61½% TiO<sub>2</sub>)
- ¾ lb. pure grained aluminum
- 55 1 lb. sodium chlorate

was ignited to produce a titanium-boron-aluminum ferro alloy by thermit reaction.

As a result of this reaction, 33 lbs. of an alloy containing 41.76% titanium, 8.13% aluminum, 2.36% boron and the remainder substantially all iron with about 4% impurities, was obtained and separated from the slag. The impurities included 2.86% silicon derived from the ferrosilicon employed in the original mixture.

A 100 lb. batch of molten, de-oxidized steel was treated by addition of 1 lb. of the alloy made according to Example 1. The alloy was added in the form of lumps which dissolved readily in the steel forming a titanium boron steel containing 0.32% titanium and 0.023% boron.

The alloy of this invention comprises titanium, boron, and aluminum with the remainder iron except for the presence of incidental impurities which may be derived from the ores and ingredients employed. These impurities may include silicon, chromium, manganese, sulphur, phosphorus and other elements which in the amounts present, have negligible effect on the useful properties of the alloy. The alloy of this invention is substantially carbon free and this element cannot be tolerated as an impurity in more than insignificant amounts for instance about 0.1%. This is necessary because the boron content of the finished steel will result in hot shortness unless the carbon in the steel is completely stabilized by titanium. Hot-short steel cannot be rolled under the usual steel mill conditions. Therefore, in order to preserve proper working characteristics in the steel, it is essential to keep the carbon content as low as possible and to insure that any amount present be stabilized by titanium. The ranges of titanium, aluminum, and boron in the alloy of this invention are critical for the introduction of the desired percentages of titanium and boron in the steel with uniform and high efficiency, and the titanium content of the alloy cannot also compensate for the introduction of additional carbon, and under these conditions, the presence of any appreciable amount of carbon in the alloy of the present invention would seriously detract from its usefulness in the manufacture of titanium-boron steel. Such incidental impurities will not generally be present in excess of about 2% except when ferrosilicon is employed in the manufacture of the alloy and under these conditions, due to the presence of silicon, will not exceed about 6%.

The alloy of the present invention permits simultaneous addition of titanium and boron to molten steel conveniently and economically by a single addition which insures ready control of the proper percentages of these metals in the finished steel. The alloy of the present invention contains sufficient aluminum to protect the titanium and boron from excessive loss by oxidation when the alloy becomes heated on addition to the molten steel, and also the presence of aluminum decreases the fusion point of the alloy and improves its solubility in the iron, to a considerable

extent. The proportion of titanium present in the alloy according to this invention is such that efficient and ready solution is obtained. Alloys containing more than about 45% titanium are difficult to dissolve in steel, while if less than about 35% titanium is present, too large an addition to steel is required to obtain the proper titanium content. Therefore, the range of titanium in the alloy of the present invention is between about 35% and 45% titanium; the boron content is adjusted so that the proper ratio of this element to the titanium is present allowing for losses in the constituents of the alloy when employed in the treatment of steel.

Employment of the single alloy of this invention has several advantages over the addition of titanium and boron as separate ferro alloys. The presence of aluminum as a constituent of the alloy assures close proximity of this metal, and therefore, more efficient protection against oxidation losses in the added elements. Furthermore, the inevitable loss of titanium which is more or less readily oxidized at the temperatures involved, is reasonably constant and the amount actually recovered can be predicted to insure the desired content in the finished steel.

This application is a continuation of application, Serial No. 95,573 filed May 26, 1949, now abandoned.

While this invention has been described and illustrated by the examples shown, it is not to be considered to be strictly limited thereto and modifications and variations may be employed within the limits of the following claims.

I claim:

1. An alloy of the class described consisting of from about 35% to 45% titanium, from about 1.5% to 2.8% boron, from about 7% to 15% aluminum, less than 0.1% carbon and the remainder iron and incidental impurities.

2. An alloy of the class described consisting of about 38% titanium, about 2.6% boron, about 14.4% aluminum, less than 0.1% carbon and the remainder iron and incidental impurities.

3. A method for production of titanium boron alloy steel which comprises adding to deoxidized steel while molten, an alloy consisting of from about 35% to 45% titanium, from about 1.5% to 2.8% boron, from about 7% to 15% aluminum, less than 0.1% carbon and the remainder iron and incidental impurities.

VIATCHESLAV V. EFIMOFF.

#### REFERENCES CITED

55 The following references are of record in the file of this patent:

#### UNITED STATES PATENTS

|              |          |                |
|--------------|----------|----------------|
| Number       | Name     | Date           |
| 60 2,295,706 | Comstock | Sept. 15, 1942 |

#### FOREIGN PATENTS

|            |               |              |
|------------|---------------|--------------|
| Number     | Country       | Date         |
| 60 561,407 | Great Britain | May 18, 1944 |